

## UNITED STATES PATENT OFFICE

2,306,872

## METHOD OF CARROTTING FUR AND COMPOSITION FOR USE THEREIN

Constantine F. Fabian, Brookfield Center, Conn., assignor to The Non-Mercuric Carrot Company, Danbury, Conn., a corporation of Connecticut

No Drawing. Application December 27, 1941,  
Serial No. 424,596

9 Claims. (Cl. 8—112)

The present invention relates to a method of carroting fur and particularly to a method which eliminates the manual labor of brushing the carroting solution upon the fur as is presently done.

The carroting of fur is well known in the art of felt making and comprises the treating of the fur with a chemical solution which renders the fur capable of felting. The chemical solutions used in the treatment above outlined are generally known as carroting solutions. Many of these carroting solutions are known, the vast majority of which are composed of mercury nitrate and nitric acid in varying proportions in aqueous solution. Recently, however, the non-mercuric carroting solutions described in Fabian Patent No. 2,169,997, issued August 22, 1939, as well as in the following patents issued to Fabian and Sachanen, No. 2,048,645, issued July 21, 1936, Nos. 2,087,854, 2,087,855, 2,087,856, 2,087,857 issued July 20, 1937, and No. 2,144,487 issued Jan. 17, 1939, have come into wide use. The method of the present invention is, however, applicable whether the carroting solution be that of the above-mentioned patents or the older mercury nitrate-nitric acid solution, or other known carroting solutions.

The present commonly used method for application of the carroting solution to the furs is, as indicated above, the brushing of the fur with the solution while the fur is on the pelt, with subsequent drying usually performed at an elevated temperature. It has been found impossible to carrot the fur by immersion either while on the pelt or after cutting the fur therefrom. Apparently fur which has been immersed in the carroting solution undergoes a chemical change throughout its length and this apparently, possibly due to the fact that strains set up in the fibres when treated for only a portion of their length are absent when treated throughout their length, prevents the subsequent felting action desired.

Such a manual method has numerous disadvantages. The brushing operation is not uniformly performed due both to variation between different operators and to fatigue. It is obvious that this lack of uniformity of treatment is important when it is considered that many fur cutting plants produce 3000 lbs. or more of carroted fur daily, which means that approximately 75,000 skins have to be individually handled in the brushing operation.

Furthermore, the drying operation as at present performed requires the stacking of the pelts, in some instances in special arrangements, for

example back to back, which is done manually and is, of course, subject to the same lack of uniformity.

Even more important than the above is the fact that when the brushing operation is performed there is danger to the operators since it is practically impossible to keep from splashing the carroting solution on the hands and face, and furthermore the fumes given off by the solution are frequently inhaled.

In the past many explanations have been given as to exactly what occurred during the carroting operation. Among the explanations was one which was based on the assumption that the fur fibres were coated with some kind of waxy material which was removed during the carroting and which made it possible to felt the fur. In accordance with this theory, attempts were made to carrot the fur by the use of mechanical forces, as for example by the employment of abrasives or metal brushes. In Tweedy Patent No. 339,349, issued April 6, 1886, it was suggested that fur could be carroted by placing it in a tumbling barrel together with abrasives in powdered form, which would remove the waxy coating and leave the fur in a feltable condition. Such a theory is at present believed to be erroneous. In any event methods such as that set forth in the above-mentioned Tweedy patent have never been commercially successful.

My present invention comprises a method whereby the carroting solution is applied to the fur while on the pelt by means of material capable of absorbing the carroting solution, mixed with material capable of carrying the first mentioned material into the fur to the desired extent, the mixture being hereinafter called a carroting mixture.

It is an object of my invention to improve the method of fur carroting and to provide a composition of matter for carrying the carroting solution into the fur to the proper extent to bring about the desired carroting effect.

It is another object of my invention to provide such a process or method whereby the time required for drying the fur after carroting is reduced to a minimum.

It is still another object of my invention to provide a process which will eliminate the brushing or spraying of the carroting solution on the skins, thereby increasing the uniformity of the carroting action and reducing the hazards and expenses involved in carroting operations.

A further object of my invention is to provide a carroting process in which the individual treat-

ment of the skins is eliminated, and replaced by treatment in volume, or mass production, thereby increasing the production rate immensely.

In my new process the carroting solution, which may be any of the known workable solutions, is applied to the fur by means of powdered or divided material which is non-reactive to the carroting solution, which is highly absorbent, and which is neutral. Examples of such materials are sawdust, natural and synthetic ground sponge, powdered asbestos, and many others.

In general, as is indicated above, the material should be in a finely divided or powdered state. These absorbent materials are wetted with the carroting solution and are then brought into contact for a predetermined period of time, variable in accordance with the type of fur being treated, with the fur while still on the pelt.

Since the absorbent materials, hereinafter called conveyors since they convey the carroting solution to the fur, are non-reactive, they do not consume the carroting solution nor any of the ingredients thereof, but rather give off the solution to the fur with which the reaction proceeds and on which the ingredients of the carroting solution are consumed. It will be obvious that the period of time during which the conveyors are in contact with the fur must be sufficiently great to give the proper carroting effect and that there is no advantage to be gained by leaving the materials in contact subsequent to the establishment of equilibrium between the moisture content of the conveyors and that of the fur.

Due to the fact that the conveyors are of a low specific gravity, they do not possess the property of penetrating into the fur on the pelts. I have found that if the conveyors, either prior or subsequent to being wet with the carroting solution, are mixed with neutral non-reactive, non-absorbing, ground materials of relatively high specific gravity, at least greater than that of water, then the conveyors are carried into the depth of the fur on the skin by these last mentioned materials, which for this reason will hereinafter be called penetrators. Examples of such penetrators are sand, ground or powdered abrasives, and ground stone not containing carbonates. Experiments indicate that penetrating capacity varies somewhat with the size of the penetrator particles, the best results being obtained with a size of from 20 to 30 mesh.

Since, as has been stated hereinabove, the carroting effect occurs only when the fur fibre has been treated with the carroting solution over a portion of its length, it is obvious that the proportion of conveyors and penetrators comprising the carroting mixture will depend upon the type and quality of the pelts. Generally speaking, the longer and thicker the fur on the skin, the larger the amount of penetrator which should be included in the mixture.

In most cases the optimum result is secured when the conveyors and penetrators are mixed in the proportion of one to one by weight. The conveyors and penetrators must be thoroughly mixed and furthermore the carroting solution must be thoroughly mixed with either the conveyor alone before its mixture with the penetrators, or with the mixture of penetrators and conveyors.

As indicated above, any of the known operable carroting solutions may be utilized. I have found, however, that the concentration of the carroting solution should be considerably higher when using my method than when using the old method of brushing. In most cases the concen-

tration has to be increased in the neighborhood of from 30% to 50%. Thus if the strength of the carroting solution measured by the Baume hydrometer is 9 degrees, when the old brushing method is utilized, the strength of the same carroting solution when used in my method should be between 11.8 degrees and 13.5 degrees.

I have further found that when my new method is utilized the addition of glue, gelatin, or furfural to the carroting solution, prior to its incorporation in the carroting mixture, considerably improves the carroting effect and produces fur with greater felting speed. It is my belief that glue, gelatin, or furfural, when added to the carroting solution, facilitates adhesion between the conveyors and penetrators thereby improving the uniformity of penetration by the conveyors into the depth of the fur.

In any event, whether this belief be correct or not, experiment has shown that the addition of the abovementioned substances does improve the action and produce a superior carroting effect. The amount of adhesives in the carroting solution may vary considerably but practice has shown that the use of from 3 to 5% by weight, based on the total weight of the ready-to-use carroting solution, produces the desired result.

The conveyors and penetrators must be thoroughly mixed and wetted with the carroting solution before utilizing them in the carroting process. While the amount of the conveyors may vary rather widely, practice shows that between 10% and 25% of the weight of the pelts to be carroted is proper; for example if 100 pounds of rabbit skins are to be carroted by my process, then between 10 and 25 pounds of conveyors are required.

The amount of the carroting solution used with the conveyors depends upon the yield of the fur from the particular pelts. Experience has shown that each gallon of the carroting solution is capable of carroting about eight pounds of fur, this again, of course, depending to some extent on the type of fur. However, in general the amount stated above is correct. For example, if 100 pounds of skins are to be carroted and the yield of fur from this type of skin is known to be about 32 pounds, then approximately four gallons of the carroting solution is required to wet the mixture of conveyors and penetrators which would in this case consist of approximately fifteen pounds of conveyors and fifteen pounds of penetrators.

While many methods might be employed for treating the skins with the carroting mixture, I have found that tumbling is a preferable method. In this method a drum which is of substantially the same construction as the drum used for softening pelts in the fur cutting industry, has placed in it the skins to be treated, preferably in alternate layers with the carroting mixture, and the drum is thereafter rotated for a period of time. The speed of the drum can vary greatly and depends upon the length and thickness of the fur on the skin, the longer and thicker fur requiring higher speed, the range however lying between 30 and 60 revolutions per minute. It is beneficial to place wooden bars between the layers of skins in the drum in order to separate the skins and increase the uniformity of the treatment of the individual skins. As with the drum speed, the time to perform the carroting operation may vary within wide limits but in general this period of time will be between three and six hours.

Subsequent to the carroting operation, with which may be combined the drying operation, the skins are placed in a second drum which has perforated sides, and are rotated therein for the purpose of shaking out from the skins the now substantially dry conveyors and penetrators which may be used again after having been wetted with a carroting solution.

While the above has described my new process, examples of the complete process are set forth below:

*Example I*

100 pounds of English unpulled skins are to be carroted. The fur yield of such skins is known to be approximately 32%. 15 pounds of the conveyor, in this instance sawdust, and 15 pounds of the penetrator, a ground abrasive, are thoroughly mixed and wetted with four gallons of the carroting solution containing 4% of adhesive in this instance gelatin. A layer of skins is placed in the drum and a portion of the prepared carroting mixture is spread on this layer of skins. The second layer of skins is then placed in the drum and spread with the carroting mixture, and this process is continued until all of the skins are in the drum and all of the prepared mixture has been used. In each instance wooden bars are placed between the layers of skins in order to separate them and facilitate the action of the carroting mixture upon the fur. After the drum has been charged, the opening is closed, and then the carroting operation is started by rotating the drum at a speed of approximately 40 revolutions per minute, this operation being continued for four hours. After the first two hours of rotation preheated and preconditioned air is introduced into the rotating drum through the normal axial opening, care being taken not to have the temperature of the air above 120° F. This introduction of preheated air into the drum facilitates the carroting effect and provides for greater uniformity thereof, and likewise causes drying of the fur so that after the four hours the skins are properly carroted and completely dry.

After the operation described above the skins are removed from the first drum and placed in the second or perforated drum. In this drum they are rotated for a period of time determined by observation. This period is sufficient to remove the dry transmitters and conveyors from the fur. After this operation the fur is completely carroted and dried and is also free from both conveyors and penetrators and ready to go to the cutting machines for the cutting of the fur from the skins in the ordinary manner.

*Example II*

100 pounds of American double ring skins are to be carroted. This type of skin is well known in the industry and is known to be one of the most difficult to carot. The yield from this type of fur is relatively high, being about forty pounds of fur from each one hundred pounds of pelts. In this instance twenty pounds of conveyors are mixed with twenty pounds of penetrators, and the resulting mixture wetted with five gallons of carroting solution. The skins and carroting mixture are placed in the first drum in alternate layers in the same manner as described in connection with Example I, and the drum is thereafter rotated at a speed of approximately 60 revolutions per minute for approximately six hours. During the first three hours of the six the carroting operation is performed and during the remaining three hours drying is effected.

As in Example I the skins are thereafter placed in a second drum and rotated for a sufficient time to separate the now dry carroting mixture from the fur after which the skins are ready for further operations in the ordinary manner.

5 While I have described preferred embodiments of my invention, it is to be understood that variations thereof may be utilized without departing from the scope of my invention. Therefore, I 10 wish to be limited not by the foregoing description but solely by the appended claims.

What is claimed is:

1. The method of carroting fur which comprises bringing said fur while on the skin into 15 intimate moving contact with a carroting mixture, said mixture comprising a relatively heavy powdered penetrating material, a relatively light finely divided absorbing material, and a carroting solution absorbed by said absorbing material, 20 both said absorbing and said penetrating materials being non-reactive to said carroting solution.

2. The method of carroting fur which comprises bringing said fur while on the skin into 25 intimate moving contact with a carroting mixture, said mixture comprising a relatively heavy powdered penetrating material, a relatively light finely divided absorbing material, and a carroting solution, including an adhesive absorbed by said absorbing material, both said absorbing and said 30 penetrating materials being non-reactive to said carroting solution.

3. The method of carroting fur which comprises bringing said fur while on the skin into 35 intimate moving contact with a carroting mixture, said mixture comprising a relatively heavy powdered penetrating material, a relatively light finely divided absorbing material, and a carroting solution including an adhesive of the group glue, gelatin and furfural in an amount in the 40 range of from 3% to 5% by weight of the carroting solution absorbed by said absorbing material, both said absorbing and said penetrating materials being non-reactive to said carroting solution.

4. The method of carroting fur which comprises placing said fur while on the skins in a 45 container, bringing said fur into moving contact with a carroting mixture, said carroting mixture comprising a relatively heavy powdered penetrating material and a relatively light finely divided absorbing material, continuing said contact for a period of from two to three hours, and thereafter continuing the movement of said skins in said 50 container while causing heated air to come into contact therewith for a period of from two to three hours to effect drying of the skins and the carroting mixture.

5. The method of carroting fur which comprises placing said fur while on the skins in a 60 container, bringing said fur into intimate moving contact with a carroting mixture, said carroting mixture comprising a relatively heavy powdered penetrating material and a relatively light finely divided absorbing material, continuing said contact for a period of from two to three hours, and thereafter continuing the movement of said skins in said 65 container while causing air heated to a temperature of not over 120° F. to come into contact therewith to effect drying of the skins and the carroting mixture, for a period of from two to three hours.

6. A carroting mixture comprising a conveyor, a penetrator, and a carroting solution, said conveyor being relatively light finely divided material 70 capable of absorbing said carroting solution and

non-reactive therewith, said penetrator being relatively heavy finely divided material capable of taking said conveyor into the depth of fur on the skin, said conveyor and said penetrator being present in such proportions that the carotting solution absorbed by said conveyor will be brought into intimate contact with the fur throughout a portion of the length of the fur fibre only.

7. A carotting mixture comprising a conveyor, a penetrator and a carotting solution, said conveyor being a material of the class sawdust, natural or synthetic ground sponge, powdered asbestos, capable of absorbing said carotting solution and non-reactive therewith, said penetrator being relatively heavy finely divided material capable of taking said conveyor into the depth of the fur on the skin, said conveyor and said penetrator being present in such proportions that the carotting solution absorbed by said conveyor will be brought into intimate contact with the fur throughout a portion of the length of the fur fibre only.

8. A carotting mixture comprising a conveyor, a penetrator, and a carotting solution, said conveyor being relatively light finely divided material capable of absorbing said carotting solution and

non-reactive therewith, said penetrator being of the class sand, ground or powdered abrasives, and ground stone containing no carbonates, capable of taking said conveyor into the depth of the fur on the skin, said conveyor and said penetrator being present in such proportions that the carotting solution absorbed by said conveyor will be brought into intimate contact with the fur throughout a portion of the length of the fur fibre only.

9. A carotting mixture comprising a conveyor, a penetrator, and a carotting solution, said conveyor being relatively light finely divided material capable of absorbing said carotting solution and non-reactive therewith, said penetrator being relatively heavy finely divided material capable of taking said conveyor into the depth of fur on the skin, said conveyor and penetrators being approximately in the proportion of one to one by weight, said conveyor and said penetrator being present in such proportions that the carotting solution absorbed by said conveyor will be brought into intimate contact with the fur throughout a portion of the length of the fur fibre only.

CONSTANTINE F. FABIAN.